

## UNITED STATES PATENT OFFICE

ALEXANDER L. FEILD, OF CANTON, OHIO, ASSIGNOR, BY MESNE ASSIGNMENTS, TO REPUBLIC STEEL CORPORATION, OF YOUNGSTOWN, OHIO, A CORPORATION OF NEW JERSEY

MANUFACTURE OF STAINLESS IRON

No Drawing. Application filed December 18, 1926, Serial No. 155,767. Renewed January 14, 1931.

This invention relates to the manufacture of those low-carbon, high-chromium steels, characterized by resistance to corrosion, tarnish and heat, and which, because of these properties and their low carbon content, are variously designated as stainless, stable-surface or rustless irons.

It has hitherto been customary in the commercial manufacture of these irons to proceed by way of the more or less obvious method of adding to a molten bath of low-carbon steel the necessary quantity of chromium as low-carbon ferro-chrome, the carbon content of the ferro-chrome being low enough to yield by carefully conducted melting operations a product of satisfactory analysis so far as carbon and chromium are concerned. In the manufacture of a stainless iron containing approximately 17% chromium and less than 0.10% carbon, it has been necessary, for instance, to use a low-carbon ferro-chrome containing not over 0.10% carbon and approximately 72% chromium.

For the manufacture of iron-chromium alloys within the stainless iron range of analysis, low-carbon ferro-chrome is a relatively expensive raw material. High-carbon ferro-chrome of the 4 to 6% carbon grade, which is used so extensively in the manufacture of ordinary chromium steels, may be had at a price, per pound of contained chromium, which is somewhere between one-third and one-half that of the low-carbon ferro-chrome. The commercial advantage of employing high-carbon ferro-chrome instead of low-carbon ferro-chrome, if a suitable method of utilizing the former could be devised, has long been apparent; and it has been equally apparent that such a process would of necessity involve decarbonization. A mixture of carbon-free iron with an amount of 4% carbon ferro-chrome sufficient to yield a 12% chromium alloy would under ideal conditions of simple melting give rise to a product containing approximately 0.68% carbon. Under similar conditions, a 6% carbon ferro-chrome, admixed with pure iron to give an 18% chromium alloy, would lead to a carbon content of approximately 1.53%. In both instances the high-carbon ferro-

chrome has been assumed to contain 70% chromium. Accordingly, in the interests of lower manufacturing costs, methods based on decarbonization and on the employment of high-carbon ferro-chrome have been proposed.

I have found by observation and experiment that such methods as have been hitherto proposed are either inoperative, or are characterized by extremely grave operating difficulties. One of the chief difficulties is the slow rate of decarbonization as the carbon content of the metal bath falls toward the low value required and the inefficacy of the procedures followed to restrain oxidation of chromium. Heats conducted in accordance with such processes are unduly prolonged, furnace refractories are subjected to severe wear and tear, slag volume tends to increase to an excessive and unmanageable degree, and high losses of chromium to the slag are unavoidable because of slag and furnace conditions unfavorable to its recovery.

I specifically disclaim as being within the scope of my invention the process which is disclosed by Shackelford, Penniman, and Cain in U. S. Patent 1,622,977, or any like process in which a ferrous metal bath in which high-carbon ferro-chrome is incorporated, or its equivalent, is brought by decarbonization under a limey or basic slag to the carbon and chromium contents desired.

My invention relates to a method for the manufacture of low-carbon, high-chromium ferrous alloys of the type known as stainless irons from chromium alloys relatively high in carbon. It relates in particular to the manufacture of commercial stainless irons, containing 12 to 18% chromium and not more than 0.12% carbon from high-carbon ferro-chrome of the 4 to 6% carbon grade, i. e. the common commercial product. This method embraces and is based upon certain new and novel features not hitherto described or employed in the art and constitutes a distinct advance in stainless iron metallurgy so far as manufacturing costs are concerned.

My method of manufacture is characterized by the following novel procedures:

(A) Completing decarbonization of the

entire charge of high-carbon ferro-chrome with from 6 to 11.5% chromium in the metal bath, as against 12 to 18% chromium in the case of prior processes, thereby decreasing by approximately one-half the retarding effect of chromium on rate of final carbon removal from the metal bath.

(B) Conducting decarbonization by means of molten iron ore or roll scale, in absence 10 of additions of lime or other basic material chemically inert so far as oxidation of carbon is concerned, as against decarbonization by means of a limey or strongly basic slag in the case of prior processes, thereby bringing 15 about rapid removal of carbon from the metal bath.

(C) Repressing chromium oxidation and its loss to the decarbonizing slag entirely by controlling within certain limits the proportion 20 of iron ore or roll scale charged.

(D) Conducting decarbonization on approximately that amount of high-carbon ferro-chrome which is required on the basis of practically complete recovery of chromium 25 in the finished product, as against conducting decarbonization on a large excess of high-carbon ferro-chrome, thereby decreasing the time and expense of decarbonization.

(E) Subjecting to a silicon reduction 30 operation a non-basic slag, high in reducible oxides and formed by the action of iron ore or roll scale on a metal bath in which high-carbon ferro-chrome has been incorporated, by means of additions of lime and ferro-silicon, thereby avoiding unnecessary dilution 35 of the reducible oxides and promoting a rapid rate and high efficiency for the reduction operation.

(F) By means of the silicon reduction 40 operation above-mentioned, returning a molten high-chromium iron-chromium alloy, substantially higher in chromium than the commercial stainless irons, to the molten low-chromium iron-chromium alloy obtained 45 at the end of decarbonization and increasing the chromium in the metal bath from an initial value of 6 to 11.5% to a final value of 12 to 18%, thereby producing the desired stainless iron product by the rapid admixing 50 of two molten iron-chromium alloys, neither of which is of commercial stainless iron type and each of which is produced under conditions which have unique advantages in regard to production economy.

(G) Obtaining the desired stainless iron 60 product under a non-decarbonizing, non-carbonizing slag and bringing the metal bath for the first time to a stainless iron composition with respect to carbon and chromium under 65 a slag of the aforesaid type, thereby insuring an accurate control of the analysis of the final product and an almost complete recovery of chromium.

My process comprises two distinct and 65 separate steps in operation. In carrying out

the first step, high-carbon ferro-chrome is incorporated in the bath under conditions which result (a) in elimination of carbon by oxidation and (b) in the distribution of the chromium originally contained in the 70 ferro-chrome between the metal bath and the slag. The second step of the process is carried out in the same furnace without removing the slag and consists in reducing the oxidized chromium from the slag by means 75 of a metallic reducing agent and recovering it in the metal bath below. In addition to the initial charge of low-carbon steel which serves as a base, the materials employed in the first or oxidizing step are high-carbon ferro-chrome and roll scale (or iron ore). In carrying out the second step, lime and a metallic reducing agent, preferably pulverized 50 per cent ferro-silicon, are the 80 raw materials.

Carbon elimination is confined entirely to the first step of the operation and is completed before lime and ferro-silicon are added. If the process is interrupted at the end of the first step, a low-carbon iron chromium alloy is obtained but at a loss of approximately 50% of the chromium incorporated in the bath, nor have I found it possible, regardless of chromium loss, to produce by the first step alone a product with a 90 sufficiently high-chromium content (12% or more) and a sufficiently low-carbon content (0.12% or less) to fall within any of the commercially accepted analysis limits for stainless iron. The second step alone makes 95 possible the attainment of an acceptable stainless iron analysis and at the same time reduces the chromium loss to such a relatively low figure that the commercial advantages of the process in competition with 10 established processes are immensely enhanced.

In order that the principles and practice involved may be more clearly understood I shall now describe in some detail how the invention has been successfully applied in 11 actual operation.

In carrying out the process I have employed a 3-ton Heroult furnace of standard design equipped with a Westinghouse automatic regulator and preferably operated with three 12-inch carbon electrodes on 3-phase current at 110-volts. The bottom lining may be of any suitable refractory. The roof is constructed of silica brick in accordance with regular practice.

Steel scrap, preferably of low-carbon content, is charged directly on the furnace bottom and melted down in absence of non-metallic or slag-forming additions of any sort. The resulting metal bath carries a light slag resulting from the oxidation of the charge but this slag, as a rule, is not sufficient in amount to cover the surface of the metal. When the bath has reached a rather high de- 12

gree of super heat (about 3250° F.) iron ore, preferably of low silica content, or clean roll scale is charged into the furnace in relatively large amount. The amount of iron ore or scale used depends primarily upon the final 5 chromium content of the stainless iron and is roughly proportional to the latter. In the manufacture of a product analyzing 16.5 to 18% chromium I have employed between 10 1400 and 1750 lbs. of roll scale per ton (2240 lbs.) of steel scrap charged or 700 to 875 lbs. per ton of stainless iron produced. The roll scale readily melts to form a fluid slag, and causes a rapid drop in the carbon content of 15 the molten steel to a very low figure (approx. 0.02-0.04% carbon) in case the scrap initially contained appreciable carbon. High-carbon ferro-chrome analyzing 4 to 6% carbon and preferably in lump form is next 20 charged into the furnace. The ferro-alloy is added gradually to avoid undue chilling of the bath and also to prevent the vigorous "boiling" action from ejecting the slag and metal through the doors. This boiling action 25 is similar both in appearance and in origin to the well-known carbon boil in the open-hearth furnace and is due to the reaction between the carbon originally contained in the ferro-chrome and the iron oxide in the 30 bath. In making stainless iron of 17% chromium and 0.10% carbon content from high-carbon ferro-chrome analyzing 66% chromium and 5.9% carbon, the total ferro-chrome charged amounts to approximately 1180 lbs. 35 per ton of steel scrap charged or to 590 lbs. per ton of stainless iron produced. The electrodes are raised during a violent boil in order to avoid undue electrode consumption and possible contamination of the bath with 40 carbon from the electrodes.

The metal bath should be maintained at a sufficiently high temperature and the slag sufficiently high in iron oxide to cause the carbon content of the metal bath to remain 45 always at a comparatively low value. Toward the completion of this procedure of charging high-carbon ferro-chrome the rate of carbon oxidation will be retarded appreciably if there is any deficiency in the amount of roll scale or ore originally charged. In such an event, a supplementary quantity of roll scale may be charged in order to bring the carbon down to the desired percentage. When the entire quantity of high-carbon ferro-chrome has been charged, the carbon content is brought down, by an ore addition if necessary, to the percentage desired in the finished product, and preferably 0.01-0.02% lower than the maximum specified. After practice has been established in the case of any particular furnace and grade of raw materials, such a supplementary ore addition is unnecessary and, in fact, becomes undesirable, since it prolongs the decarbonizing period.

The oxidizing slag which originally consisted of molten ore or scale contains at the completion of the first step of the process 70 chromium oxide and silica as essential constituents in addition to iron oxide. The chromium oxide is derived by oxidation from the chromium contained originally in the high-carbon ferro-chrome. The silica is derived in part from the silicon contained in the high-carbon ferro-chrome, in part from 75 the silica content of the ore or scale, and in part from drippings from the silica roof. Since a low silica content is desired in the oxidizing slag, I prefer to employ a high-carbon ferro-chrome which does not exhibit an 80 unduly high silicon content. For the same reason, I prefer clean roll scale to iron ore; the latter when used should be low in silica. To avoid excessive drippings from the silica roof which are possible at the high temperature at which the bath is worked during the 85 oxidizing period, I prefer not to prolong this period of operation beyond the minimum time required. The oxidizing slag at the conclusion of the first step will generally contain 5 to 20%  $\text{SiO}_2$ , 0 to 15%  $\text{CaO}$ , 3 to 15%  $\text{Al}_2\text{O}_3$ , 1 to 3%  $\text{MnO}$ , 0 to 5%  $\text{MgO}$ , and from 90 45 to 80% of the oxides of iron and chromium combined. There is a consistent increase in the total amount by weight of chromium 95 oxide in the slag throughout this period of operation, but the actual percentage at any particular time depends largely on the manner in which the ore or scale is added.

I am of the opinion that, when high-carbon ferro-chrome is added to the bath, a large proportion of its contained carbon may be oxidized and escape as a gas, concurrently 100 with the melting of the lumps of ferro-chrome, without actually becoming thoroughly incorporated and dissolved in the metal bath. Oxidation of the chromium content of the ferro-chrome probably proceeds side by side with the oxidation of carbon, so that a part of the chromium may 105 never become diffused through the metal bath. When the iron oxide content of the slag becomes relatively lowered due to its reaction with the metal bath and entry of chromium oxide into the slag, both carbon 110 and chromium from the high-carbon ferro-chrome are retained by the metal bath more tenaciously than when the percentage of iron oxide in the slag is at a higher value, this increase in resistance to oxidation being 115 greater in the case of carbon than of chromium. In other words, by means of the procedures which constitute the first step in operation, the proportion of chromium which is oxidized and passes into the slag increases 120 rapidly as the carbon content of the metal bath is lowered. When the carbon in the metal is finally brought down to 0.10%, it will be generally observed that approximately one-half by weight of the chromium added 125 130

as ferro-chrome has been oxidized and entered the slag in making a stainless iron which is to finish at 0.10% carbon and 17% chromium.

- 5 No evidence has yet been obtained in support of the theory that carbon in the metal bath reacts at any stage of the process with the chromium oxide content of the slag with a resultant reduction of chromium into the metal bath. Operating data prove conclusively that such a reaction never proceeds and there are good theoretical grounds for concluding that it cannot proceed under the operating conditions which characterize this 10 process. The total weight of chromium in the metal bath during the oxidizing period never suffers an increase except what is due directly to an addition of high-carbon ferro-chrome.
- 15 20 Analyses of samples taken from the metal bath at various times during the oxidizing period of representative heats, together with the chromium oxide and iron oxide content of several slag samples taken at the particular times in question are given below:

| 30 | Metal bath |          | Slag                           |                                |
|----|------------|----------|--------------------------------|--------------------------------|
|    | Carbon     | Chromium | Cr <sub>2</sub> O <sub>3</sub> | Fe <sub>2</sub> O <sub>3</sub> |
|    | Per cent   | Per cent | Per cent                       | Per cent                       |
|    | .05        | 6.95     | 22.73                          | 21.92                          |
|    | .055       | 5.44     | 21.00                          | 35.52                          |
|    | .08        | 7.43     | 42.68                          | 18.88                          |
|    | .10        | 8.64     |                                |                                |
|    | .11        | 8.90     |                                |                                |
|    | .125       | 10.7     |                                |                                |
| 35 | .13        | 11.9     | 30.95                          | 10.56                          |
|    | .14        | 13.47    |                                |                                |
|    | .15        | 15.30    |                                |                                |
|    | .18        | 17.09    |                                |                                |

40 The tabulated data above indicate clearly what importance attaches to each 0.01% of carbon within the stainless range. It is readily possible to manufacture by my oxidizing step alone an alloy analyzing 17% chromium and 0.17-0.18% carbon and with a loss 45 of added chromium amounting to only about 30%. In going to an alloy of 0.10% carbon content, the maximum chromium obtainable in such an alloy by my oxidizing step alone is in the neighborhood of 10%, with a loss 50 of added chromium amounting to approximately 50%.

I now come to the second step of the process. This stage of operation is begun with a highly heated metal bath above which is a 55 slag containing chromium oxide and iron oxide as essential constituents. The metal bath should contain 6 to 11.5% chromium and not more than 0.12% carbon. The chromium oxide content of the slag is derived, by 60 oxidation during the first step of operation, from the chromium originally contained in the high-carbon ferro-chrome. The addition agents used during the second step of operation are burnt lime (CaO) and pulverized 65 ferro-silicon. The exact manner in which

these additions are made may be varied at will to a considerable degree. However, I prefer to make an initial addition of lime which is spread over the surface of the bath. A mixture of lime and pulverized ferro-silicon is then fed gradually into the bath, preferably around or beneath the electrodes. The pulverized ferro-silicon reduces the chromium and iron oxide contained in the slag and forms silica, which acidic oxide is in turn 70 neutralized, or else combines with, the lime present. As a result, the slag which at the beginning of this operation was black or dark brown in color due to its high percentage of iron and chromium oxides gradually verges 75 towards a basic character and acquires a lighter color. High recoveries of chromium may be obtained without actually converting the original black slag into a greenish or greyish-white basic slag of the disintegrating 80 type. The ratio of lime to ferro-silicon (50%) which leads to the best results lies between 1.5 and 3.0. The weight of burnt lime used will as a rule amount to from 375 to 750 lbs. per ton of metal produced. At the completion of the second step, or reducing period, of operation the slag should not contain more than 2% oxide of chromium and 2% oxide of iron. If the reduction process is not efficiently conducted, however, these percentages will be higher. The amount of residual chromium oxide in the slag corresponds to the net loss of chromium for the operation as a whole. The silica (SiO<sub>2</sub>) content of the slag at the end of the reducing period lies as a rule between 25 and 35%.

Since the metal bath at the end of the oxidizing period contains a substantially lower percentage of chromium than that required in the stainless iron product, it is a requirement of my method of manufacture that the metal returned to metal bath from the slag by silicon reduction must be of sufficient total weight and sufficiently high in its percentage of chromium to enrich the decarbonized metal in chromium to the desired degree. In order that this requirement be met, the relative proportions of iron or steel scrap, high-carbon ferro-chrome, and iron ore or roll scale incorporated in the bath prior to silicon reduction must be carefully adjusted in the manner already described above. When a reducing agent containing 50% iron, such as ordinary 50 per cent ferro-silicon, is employed, the metal returned to the metal bath contains roughly 35% chromium.

The metal bath at the completion of the reducing period should be low in silicon, and as a rule does not exceed 0.04-0.05%. Reduction of chromium and iron oxides by the silicon contained in the pulverized ferro-silicon occurs, to all practical purposes, entirely within the slag layer, the reduced metals finding their way subsequently into the metal bath. The introduction of lump ferro-sili-

con into the metal bath for reduction purposes, while not beyond the scope of the invention, is not the preferred practice. When the silicon content of the metal bath is increased by additions of lump ferro-silicon before reduction of chromium oxide from the slag is practically complete, the carbon content of the metal bath is inclined to rise and its chromium content to fall appreciably.

10 Whereas the second step of operation is designated as a "reducing" step, this term refers only to the action of the silicon content of the ferro-silicon in reducing the oxides of iron and chromium from the slag. The slag itself is never of a reducing type at any stage of the second period. When reduction by silicon is complete, the slag corresponds to a neutral or basic calcium silicate slag. Before reduction by silicon is completed or

20 when this reduction is incomplete, the slag contains the oxides of iron and chromium and remains of an oxidizing type within the generally accepted meaning of the term. Employment of pulverized coke or calcium carbide to assist in reducing the oxides of chromium and iron from the slag and simultaneously to "refine" the metal is unnecessary and, according to my particular experience, almost invariably increases the carbon content of the metal bath.

30

When it is desired for any reason to finish the heat under a new slag, thus continuing the operation beyond the completion of the second period, it is preferred (a) to remove all or the major portion of the calcium silicate slag, which is formed during the second period and which attains to a considerable volume before reduction is completed, (b) to add sufficient lump ferro-silicon to raise the silicon content of the metal bath up to 0.30-0.40%, and (c) to build up a normal volume of basic calcium silicate slag by means of lime and powdered ferro-silicon (or sand) in the usual way. This procedure is well-known in the art and regularly employed in electric furnace practice so that it need not be considered as a novel or essential feature of the present invention. It is employed to particular advantage during the period when the furnace is being held up prior to tapping on a preliminary analysis for chromium in the metal bath. When the product is being made to narrow specification limits as to chromium, it is frequently necessary to increase the chromium percentage of the metal bath by a per cent or a fraction thereof by means of a small addition of low-carbon ferro-chrome or to lower the chromium content in the same way by an addition of low-carbon steel or ingot iron. When the metal bath is adjusted to the desired analysis as to carbon and chromium, temperature tests are made to determine whether or not the metal bath is at a proper tapping temperature (about 3000° F.). If too hot, additions of

cold stainless iron scrap may be employed to cool the bath rapidly to the desired temperature. If too cold, the power is again applied. As a rule, however, the bath will be found to be on the hot side, which circumstance provides an economical outlet for an appreciable quantity of stainless iron scrap.

5 As soon as the second step of operation is completed and the heat brought to the proper analysis and temperature, the metal may be tapped into a ladle, the specified content of silicon and manganese introduced by ladle additions of ferro-silicon and low-carbon ferro-manganese, respectively, and the ladle metal poured into ingot molds or castings in the customary manner.

10 The product which is obtained by this process is sound and free from blow-holes when cast into ingots even when the silicon content is 0.04% or less. In this respect the product differs markedly from all other stainless irons regardless of the process by which they are obtained. One of the outstanding difficulties hitherto encountered in the manufacture of stainless iron has been that of degasifying the final product so that it solidifies into an ingot free from blow-holes. This undesirable property of ordinary stainless iron does not exist in the case of my product. Silicon above 0.04% in the finished product need be added only for the purpose of meeting chemical or physical specifications. This peculiar freedom from gas evolution during solidification characterizes this chromium-iron alloy throughout the process of manufacture. A sample taken from the furnace at the completion of the first or oxidizing period freezes quietly to a sound ingot or test-piece, just as does the finished product, without any deoxidizing or other additions whatever being made.

15 I have described in detail the procedure which I now prefer to follow in conducting my process for the manufacture of stainless iron alloys, but I do not wish to limit the scope of the invention to the particular procedure outlined. I may, for instance, if I so desire, melt up all or a portion of the iron ore (or scale) and the high-carbon ferro-chrome with the initial steel scrap charge in a single melting-down operation. Again, the iron ore (or scale) and high-carbon ferro-chrome may be added to the bath alternately in lots of any convenient weight. Another variation, which I have actually employed in practice, consists in operating with not simply one oxidizing and one reducing period but two or more such cycles. Instead of ferro-silicon as a reducing agent, I may, if desired employ any one of several other well-known metallic reducing agents, such as silicon metal, aluminum, calcium-silicon, ferro-aluminum, silicon-zirconium, etc., without departure from the invention. I prefer to conduct both the first and second periods of

the process in absence of any added flux or similar slag-forming ingredients but realize that the process may be worked satisfactorily in the presence of moderate amounts of such fluxes as fluorspar, rutile, sand, soda, manganese oxide, etc.

5 The product is usually made to a specified silicon and manganese analysis but may be modified in its composition by the addition of various alloying elements such as nickel, copper, molybdenum, vanadium, etc.

10 By means of the process of the present invention I am able to produce a rustless or stainless iron within the usual limits of 0.07 to 0.12% carbon and 12.00 to 18.00% 15 chromium by the use of a high carbon ferro-chrome, with a chromium loss of 10% or less, and at a cost appreciably less than the cost of the same iron made with low carbon ferro-chrome.

20 I claim:

1. A process for making stainless iron which comprises the steps of forming a highly heated bath of a ferrous base metal, 25 charging iron oxide, removing carbon from the metal by oxidation at relatively high temperature, charging high carbon ferro-chrome, maintaining the bath at or above said high temperature to oxidize carbon from the bath, 30 charging a silicon reducing agent and lime, and maintaining the bath at high temperature until the slag is substantially free from iron and chromium.

2. A process for making stainless iron 35 which comprises the steps of forming a highly heated bath of a ferrous base metal, charging iron oxide, removing carbon from the metal by oxidation, charging high carbon ferro-chrome, maintaining the bath at a 40 temperature of approximately 3250° F. until the metal contains not more than 0.12 per cent carbon, charging powdered ferro-silicon and lime, maintaining the bath at a relatively high temperature until the slag is substantially 45 free from iron and chromium, and cooling the metal to the desired tapping temperature.

In testimony whereof I affix my signature.  
ALEXANDER L. FEILD.

50

55

60

65